# EUROPEAN PATENT SPECIFICATION

(11) **EP 2 358 942 B1**
(45) Date of publication and mention of the grant of the patent: **18.05.2016**
(21) Application number: 09756797.8
(22) Date of filing: 05.11.2009
(51) Int. Cl.: D21H 19/24, D21H 19/58, D21H 19/82, D21H 23/22

(54) **COATED RECYCLABLE PAPER OR PAPERBOARD AND METHODS FOR THEIR PRODUCTION**
BESCHICHTETES RECYCLISIERBARES PAPIER ODER KARTON UND VERFAHREN ZUR IHRE HERSTELLUNG
PAPIER OU CARTON RECYCLABLE ET PROCEDE POUR SA FABRICATION

(30) Priority: 07.11.2008 US 112526 P
(43) Date of publication of application: 24.08.2011
(73) Proprietor: Premium Board Finland Oy, 73500 Juankoski (FI)
(72) Inventor: RONKA, Johanna, Sirkku, FIN-02630 Espoo (FI)
(74) Representative: Ilgart, Jean-Christophe
(86) International application number: PCT/IB2009/007415
(87) International publication number: WO 2010/052571

(56) References cited:
- EP-A1- 1 249 533
- EP-A1- 1 659 219
- WO-A1-94/26513
- WO-A1-2008/118284
- GB-A- 1 234 880
- GB-A- 2 433 450
- JP-A- 6 123 100
- US-A1- 2005 112 387

## Description

This invention relates to coated recyclable paper or paperboard products and methods for their production. More particularly, paper or paperboard is coated with a polymer emulsion in one or more coating stations which are off-line from the paper or paperboard machine. The coating compositions and process of the invention are effective for providing coated paper or paperboard products with enhanced barrier properties.

### BACKGROUND

Coated paper and paperboard products having barrier properties are of great importance for packaging food or other products that are sensitive to environmental influences. Desirable barrier properties include grease resistance and low water penetration, as well as a smooth and uniform surface finish. In many applications the coating is also heat sealable. Known coating methods include dispersion coating, in which coating compositions of water soluble dispersion polymers, pigments and other agents are applied to the substrate using coating techniques such as blade coating, bar (rod) coating, reverse roll (film) coating, or air knife coating. Premixed coatings available from a number of coating suppliers are applied to the paperboard web at the paperboard machine. The use of premixed bulk coating compositions limits the degree to which coating compositions can be custom designed to achieve the barrier and other properties desired for a particular packaging or other product. Typically paper and paperboard are produced with the machines, where coating is performed on coating stations that are directly integrated with the paper or paperboard machines. Using in-line coating, the paperboard web is at an elevated temperature when the coating is applied, which results in greater penetration of the coating into the paperboard and a lower effective coating thickness and makes it difficult to consistently achieve the desired coating properties at the minimal cost. Because in-line coating systems are tied to the paper or paperboard production process, they are relatively inflexible and are not easily adapted for smaller production runs of, for example, specialty coated paperboard products to be manufactured in relatively small production runs.

Conventional production methods utilizing in-line coating systems have additional drawbacks of difficulty in designing and testing new coating formulations during paper or paperboard production runs, and difficulty and expense of modifying existing equipment to provide for specialty products such as products that include multiple coating layers of the same or different coating compositions. An improved system and processes is needed that can easily and economically be adapted to provide a wide variety of coated paper and paperboard products having a range of desired barrier properties. Such processes should be capable of economically producing both large and small quantities of high quality dispersion coated paper and paperboard products that are optimized to meet the particular needs of the finished product. Further, coating compositions and processes are needed that provide desired barrier properties while at the same time improve the capacity to recycle waste paper and paperboard products in order to reduce both production costs and the environmental impact of the manufacturing process and finished products.

WO 94/26513 discloses a method for manufacturing a recyclable paper stock useful as a food package or beverage container, in which at least one surface of a substrate is coated with a water based emulsion coating comprised of an acrylic-styrene copolymer and a wax.

### SUMMARY

A highly adaptable production system and method is provided for producing a wide range of high quality coated recyclable paper or paperboard for use in a variety of applications. To enable further flexibility, coating compositions are applied to paper or paperboard at one or more coating stations that may be offline from the paperboard manufacturing unit yet preferably located in the same manufacturing facility. Thus, the paper or paperboard web is cool at the time of coating application, which affords better control of the coating process and lowers the amount of coating needed to achieve desired barrier properties. Because the coating step may be decoupled from the paperboard manufacturing, the coating speed and other conditions can be controlled as necessary independent of the operating parameters of the paperboard manufacturing machine. The system is easily adapted for producing multi-layer products by providing multiple on or off-line coating stations in series and intermittent drying stations to dry the coating before the next coating is applied. The system also includes a final drying station after the last coating station and then a cooling station to cool the coated paper or paperboard to prevent the heat sealable surface from sticking when the product is rolled onto reels for storage.

An improved process for producing coated paper or paperboard products is also described. A mixing system is provided for combining water based polymer emulsions, pigment and optional additives in ratios selected to achieve desired solids content, solids dispersion, viscosity and other properties required to achieve desired coating barrier and other properties. Thus, a wide range of specific coating compositions can be prepared on site, which affords greater flexibility in the properties and performance of the finished product as compared to systems that are limited to using those coating compositions which are generally available from industrial coating suppliers.

Coating compositions are provided that include, for example, about 70 to about 90 weight %, based on the dry weight of the coating, of a water based polymer emulsion, and about 10 to about 30 weight %, based on the dry weight of the coating, of pigment. Additives such as defoamers, dispersing agents and thickeners may also be included. Such coatings may have a viscosity of about 400 to about 1000 mPas and a solids content of about 40 to about 60 weight percent, based on the weight of the coating. In another aspect of the invention, one or more dispersion polymers are included in a first coating composition for providing good grease resistance, a second coating composition is prepared to provide good water resistance properties, and a third coating composition may be provided as a precoating to provide a moisture vapor barrier and some grease resistance. These coatings may then be applied in various combinations to provide a multi-layer coated paper or paperboard having a desired range of barrier properties.

The aqueous coating is applied to the paper or paperboard. Preferrably, the paper or paperboard has a temperature of 40°C or less on at least one side. The aqueous coating is dried to provide a coated paper or paperboard. The coated paper or paperboard is cooled. Cooling may be done by air cooling or by contacting the coated paper or paperboard with a cylinder to provide a coated paper or paperboard having a temperature of 40°C or less. The cooled coated paper may be further processed with calandering.

The methods described are effective for providing a coated paper or paperboard product. The coated paper or paperboard product includes a paper or paperboard layer coated on at least one side with a first coating layer formed from a first acrylic polymer emulsion. The coated paper or paperboard product also includes a second coating layer which contacts the first coating layer. The second coating layer includes a second coating layer formed from a second acrylic emulsion. The coated paper or paperboard product has a water resistance of below 10g/m² measured with Cobb water absorption test (time 30 minutes per ASTM D 3285), moisture vapor resistance (MVTR-value per ASTM E 96) of below 120 g/m² in 24 hours (temperature 25°C, relative humidity 75%) and provides a grease penetration of 0 after 15 minutes at a temperature of 200°C (per a baking test described herein in Example 4). Furthermore, the coating retains its barrier properties of water resistance and moisture vapor resistance at temperature of 220°C. The coating or any substances in the coatings does not migrate to food in contact with the coating (as determined per European FDA test method BfR XXXVI and BfR 70XXXVI/2). At the same time coating is heat sealable with pressure of 80-100psi (551-689 kPa) and temperature of 160-200°C and time of 1-1.5 seconds.

In another aspect, the coated paper or paperboard product includes a paper or paperboard layer coated on at least one side with a first coating layer formed from a styrenebutadiene polymer emulsion. The coated paper or paperboard product also includes a second coating layer which contacts the first coating layer. The second coating layer includes a second coating layer formed from an acrylic emulsion. The coated paper or paperboard product has a water resistance of below 7g/m² measured with Cobb water absorption test (time 30 minutes), moisture vapor resistance (MVTR-value) of below 30 g/m² in 24 hours (temperature 25°C, relative humidity 75%) and provides a grease penetration of 0 after 15 minutes at a temperature of 200°C. Furthermore, the coating retains its barrier properties of water resistance and moisture vapor resistance at temperature of 220°C. The coating or any substances in the coatings does not migrate to food in contact with the coating. At the same time coating is heat sealable with pressure of 80-100psi (551-689 kPa) and temperature of 160-200°C and time of 1-1.5 seconds.

In another aspect, paper or paperboard may include multiple coating layers. The second coating layer can be applied after the first layer is dried. The cooling and calandering is done after the last coating layer. There is no upper limit, but in practice three layers is maximum for bigger volumes. A first layer can be added on a board machine by surface sizing. Then two additional layers may be added with the board machine. These three layers go to the reverse side of the board to give barrier properties. Coating layers may all include the same polymer emulsion or each coating layer may be formed from a different polymer emulsion. Different coating layers may be utilized to provide various coating properties to an end product.

In another aspect, paper or paperboard may be coated on both sides. Each side may include a single or multiple coating layers. For example, products made in accordance with the invention may include heat sealable barrier coatings on one side and one or more pigment coatings on the opposite side. In one preferred approach, multiple off-line coating stations are provided on each side of the paperboard such that one or more identical or different coating compositions may applied in layers on each side during a single production run.

In yet another aspect of the invention, the coating compositions are formulated such that trim waste and other waste generated during the coating process may be recycled to the paperboard production process without the need to first separate the applied coating or coatings from the substrate. It has been found that the compositions of the invention permit such material to be reused in the paperboard pulping process without having an adverse effect on the resulting paperboard. Preferably, the off-line coating stations are co-located at the paperboard manufacturing facility to minimize the cost of transporting the waste paper to the paper manufacturing system.

### BRIEF DESCRIPTION OF THE DRAWINGS

Figure 1 is a flow diagram generally illustrating a process for manufacturing coated recyclable paper or paperboard.
Figure 2 illustrates off-line coating machines.
Figure 3 shows a coated paperboard product.

### DETAILED DESCRIPTION

A flowchart generally describing a process for manufacturing coated recyclable paper or paperboard is illustrated in Figure 1. Figure 2 illustrates in more detail the overall system and process of a preferred embodiment of the invention that incorporates coating stations into the process. As generally described in Figure 1, paper or paperboard is produced by a baseboard machine 20 in a conventional manner. Uncoated paper or paperboard and coating compositions are supplied to one or more off-line coating machines 60. The coating process includes applying the polymer emulsion coating to at least one surface of the paper or paperboard. Water present in the polymer emulsion is removed in one or more drying stations, followed by subsequent cooling of the finished product.

### Paper and Paperboard

Baseboard machines know in the industry may be utilized to produce paper or paperboard. For example, one type of baseboard machine that may be used is manufactured by Ahlstrom. Baseboard machine may be operated using parameters commonly known in this industry. The baseboard machine 20 provides surface sizing and calandering of the paper or paperboard to provide a substrate having desired thickness, grain density and smoothness. Unlike conventional systems for producing coated paper and paperboard products, the paper or paperboard manufacturing system of the present invention is preferably not utilized for coating operations.

A wide range of uncoated paper or paperboard produced in the baseboard machine may be used for subsequent coating. Any type of fiber based material may be coated, such as for example bleached or unbleached, hardwood or softwood, virgin or recycled, uncoated forms of paper or paperboard. The basis weights of the paper or paperboard produced are preferably in the range of 80 to 300 lbs per 3.000 sq. ft. (130-500 g/m²), and have a thicknesses range from 0.008 to 0.025 inches (0.2-0.6 cm).

Paper or paperboard is prepared to provide constant surface properties which are effective for minimizing water penetration. In this aspect, paper or paperboard is sized to provide a Cobb Value of 40g/m² (60 seconds) or less. Preferably there are no fluorochemicals used in the paper or paperboard to improve grease resistance.

### Coating Compositions

A coating composition is provided for coating paper or paperboard. The coating composition is an aqueous dispersion of synthetic polymers and pigment. The synthetic polymers are generally used as binders to fix the pigment to the paper or paperboard. As used herein, "polymer emulsion" generally refers to raw materials for a dispersion. As further used herein, "polymer dispersion" refers to a coating liquid after mixing the polymer emulsion with pigment and additives. A dried finished coating is considered a "dispersion coating."

Coating composition may include from about 70 to about 90 weight %, based on the dry weight of the coating, of synthetic polymer emulsion, and from about 10 to about 30 weight %, based on the dry weight of the coating, of pigment.

Synthetic polymers that may be utilized to form water based emulsions include acrylic polymers, acrylic copolymers, copolymers of styrene and butadiene, vinyl acetate polymers, polyvinyl alcohol, poly-ethylene vinyl acetate, polyethylene vinyl chloride, polyvinylidiene chloride, and mixtures thereof. Examples of suitable acrylic and/or methacrylic acid esters include ethyl acrylate, methylmethacrylate, butylacrylate, 2-theylhexyl acrylate, methylacrylate, ethylmethacrylate, and the like, and mixtures thereof.

The pigment may be selected from any pigment useful for substrate coating compositions. Exemplary suitable pigments are aqueous dispersions of coating grade clays, such as kaolin clays, titanium dioxide, calcium carbonate, barium sulfate, talc, zinc sulfate, aluminum sulfate, calcium oxide reaction products, lithopone, zinc sulfide, other coating pigments, other similar materials, and mixtures thereof. In one aspect, pigments that may be utilized include talc and clays.

In one aspect, talc is utilized as the pigment. Talc may be added as a dry powder or granules containing 5-15% of water instead of a slurry containing 55-65% water. Addition of talc as a dry powder provides a higher solids content and higher viscosity while minimizing the amount of any thickeners needed and more importantly minimizing the amount of drying capacity and energy needed.

Coating composition will have a viscosity of about 400 to about 1000 mPas and a solids content of about 40 to about 60 weight percent, based on the weight of the coating.

The coating composition may include additives. Additives may include thickening agents, defoaming or antifoaming agents, dispersing aids, additional pigments, crosslinking agents, slip additives, release agents and antiblocking agents. Preferably there are no fluorochemicals used in the paper or paperboard to improve grease resistance.

Coating compositions are prepared in coating preparation tanks 40 by blending polymers, water, pigments and optional additives to form a dispersion. Mixing is typically conducted for about 20 to about 30 minutes. Viscosity may be adjusted with addition or water or thickening aids. The polymer emulsion may be stored in storage tanks or transported directly to an off-line coating machine 60. The coatings are preferably mixed just before use so as to have optimal properties and avoid the adverse effects of pigment coagulation and sedimentation that may occur over time. If stored, the coating compositions are preferably agitated by a mixer and/or recirculation to minimize sedimentation.

### Coating Application

Paper or paperboard may be coated with off-line or in-line coating stations. In a system using in-line coating stations, the coating station(s) are located on the paper or paperboard machine. In an off-line coating system, the coating station(s) are on a separate machine. As shown in Figure 2, the preferred embodiment of the system of the invention includes at least one, and preferably multiple, off-line coating stations 210, 212, 214 and 216 co-located at the same facility as the paperboard manufacturing system. As used herein "off-line" refers to a coating machine that can be operated independently of the baseboard machine and is not required to be in the same production line. The off-line coating machine may be located in the same factory as the machine that provides the paper or paperboard substrate. The use of an off-line coating machine is effective for providing more optimal coatings. For example, in in-line coating, the paper or paperboard substrate is hot when coating is applied. Coatings penetrate a higher temperature substrate more than a cool substrate. The increase coating penetration results in a lower coating thickness and a poorer quality and higher costing product. The use of the off-line coating machine allows the paper or paperboard to reach a temperature of 40 °C or less prior to coating. The paper or paperboard may be held for a sufficient time to cool it or it can be cooled by blowing cool air over the web. A cooling station 220 may be added to cool the paper or paperboard more quickly in advance of another coating station. Thus, it has been found that higher quality coatings can be applied at a smaller coating amount on the cooled substrate as compared to in-line coating directly onto the hot web of the baseboard manufacturing machine.

Paper or paperboard is preferably cooled to a temperature of less than about 40°C prior to coating, and most preferably about 30 °C. Cooling may be accomplished for example by blowing cool air over the web or keeping the paper or paperboard reel in room temperature long enough for it to cool down. Paper or paperboard may be supplied to a coating station from a paper or paperboard roll 200 as shown in Figure 2. Coating compositions may be applied to at least one surface of the paper or paperboard by any known means, such as by air knife, blade coating, metering roll coating, gravure coating, rod coating, curtain coating and spraying. In an important aspect, coating layers are metered onto the paper or paperboard with a rod/bar which is effective for providing a more even coating thickness. Coating amount of each layer applied with a rod/bar will be from about 5 g/m² to about 10 g/m² with a variation in thickness of 1 g/m² or less over a surface of the coated substrate. Grooved rods are especially effective for applying coating compositions to paper of paperboard. The size of the grooves is selected to give 5-10 g/m² coating weight for each layer with specific coating mixture in question. The solid content, viscosity and other reological properties of the coating influence on groove size selection. Typically rods are surface treated with chrome and have diameter of 10-15mm.

As shown in Figure 2, a topside precoating may be applied in a coating station 200. Drying stations 230 are preferably located in between each successive coating station to reduce the water content of the coating before the next coating is applied. Drying of the coatings is accomplished with hot air directed to the coated paper or paperboard web. Heated air is provided using known techniques, such as for example, propane heat. Air is continuously recirculated with removal of moisture. In this aspect, heated air having a temperature of about 100 to about 150 °C is provided to the paper or paperboard web such that the temperature of the web does not exceed about 110 °C. In one aspect of the invention, the temperature of the web after the first coating station is from about 80 to about 90 °C and after a second set of coating and drying stations is from about 105 to about 110 °C. Web temperatures may be determined at multiple locations, such as for example at a web temperature measuring point 240. Alternatively, heating stations 230 may also be modified to provide cooling, such as for example, using cooled air.

The water based emulsion coatings have dry coating weights in the range of 5 to 15 g/m², typically 7 to 8 g/m² in one layer. Drying temperatures and line speeds are dictated by the drying characteristics of specific coating formulations, for example the % solids content, substrate basis weight and absorptivity, and equipment characteristics. The amount of coating applied may be measured at coating measuring points 250. Drying conditions should be controlled to prevent blistering of the coating and roll blocking or picking of the coating during rewinding of the coated substrate or delaminating of the paperboard.

In another aspect, each side of the paper or paperboard may include multiple coating layers. These layers may be applied by using multiple off-line coating stations, for instance two for each side, 210, 212, 214, and 216 as shown in Figure 2, but the amount may also be larger. Each coating station may be used to coat the same or a different polymer dispersion than the first coating machine.

Generally, the first layer is optimized to provide optimal grease resistance and moisture barrier properties and the second layer serves to provide additional water barrier properties and to provide a heat sealable surface. However, other approaches are also possible within the scope of the invention herein.

The system preferably includes multiple coating stations effective for independently coating both sides of the substrate with one or multiple layers in same production run. The desired coating composition is supplied to the particular coating station at which it is to be applied. Thus, for example, the system may be provided with two coating stations for applying two successive pigment layers suitable for surface printing on a first side of the substrate, and two additional coating stations provided for coating the opposite second side of the substrate with two barrier layers for providing adequate grease and moisture resistance and heat sealable properties. Due to the use of off-line coating stations, such a system can be readily adapted for providing greater or fewer layers on either or both sides of the substrate by simply adjusting the number of coating stations utilized, without the need to reconfigure the paper or paperboard manufacturing machine. Coating compositions themselves can also easily be altered at the mix stations to vary the properties of each layer. Thus, a wide array of specialty designed products can be manufactured because changing from one product to another is a relatively simple operation and does not require changing the configuration or operations of the paperboard manufacturing machine.

The use of off-line coating stations has the further advantage of enabling coating of paper or paperboard produced by remote facilities.

In another aspect, coating thicknesses are measured using IR-spectroscopy. The on-line IR-spectroscopy measurement allows for continuous monitoring of coating thicknesses so that operational parameters can be adjusted as necessary to consistently achieve the desires coating thickness. Preferably, the amount of each applied coating layer can be measured in order to achieve similar barrier and other properties in every production run and avoiding the cost of using excess coating. Measuring may be conducted at measuring points 250 shown in Figure 2.

After the one or more coating stations, the coated paper or paperboard is dried in another drying station and then cooled before reeling on a cylinder. Cooling of the coated and dried paper or paperboard is done using cool air and cooling cylinders, where water is circulated inside a cylinder rolling against the web (shown as 220 in Figure 2). The cool water is directed in from the other end of the cylinder and out from the another. There are two cooling cylinders, one on each side of the paper or paperboard web. Cooling is effective for providing a coated paper or paperboard with a temperature of 40 °C or less. Proper drying is necessary to achieve good film formation and good barrier properties while avoiding sticking of the heat sealable coatings in the reels, also known as "blocking." The cooling conditions are selected to stop the drying at the correct stage so as to avoid complete drying so that the coating is heat sealable, while providing sufficient drying to prevent blocking,

After cooling, the coated paper or paperboard may be calandered.

Further advantages of the system and process of the invention reside in the fact that all coated paperboard waste from the process may be recycled directly to the paper or paperboard manufacturing process without separating the coating prior to recycling. In this aspect 100% of the coated paperboard waste is recycled. In this regard, it is preferably that the coating compositions utilized contain no detectable levels of waxes. Although waxes are typically used in many coating to improve water resistance and to provide a vapor barrier, waxes have a negative effect on recycling as they cause stickies in the recycled pulp. The compositions described herein are suitable for providing excellent barrier properties without the need for wax components. When coating is performed in the same mill where the paper or paperboard is produced, transportation costs for transporting coated paperboard waste is reduced.

### Coated Paper or Paperboard Products

Coated paper or paperboard products produced in accordance with the process described herein are compostable and recyclable without separating the coating. The coated paper or paperboard products may be used to provide moisture resistance and grease resistance. The coated paper or paperboard products are heat sealable and can be microwaved. Coating paper and paperboard products may be used for a variety of food packages such as for example bakery packaging, salad trays, frozen food containers, sandwich packaging, candies and gum.

Figure 3 generally illustrates a coated paperboard. As illustrated in Figure 3, the paper or paperboard product may include a baseboard middle layer 110. The baseboard middle layer 110 generally includes mechanical pulp and mill pulp and may include chemical pulp regions either side of the middle layer resulting from a bleaching process. The mechanical pulp in the middle layer provides bulk, while the chemical pulp layers provide flexibility as well as higher whiteness. The baseboard can also be produced totally from chemical pulp, or can contain recycled pulp. Also paper can be used as base material to be coated.

The baseboard middle layer 110 may be coated on one side with a pigment pre-coating layer 120 and a pigment top-coating layer 121 . These layers offer good surface printability. By providing two pigment layers, the coating can be provided more evenly with fewer variations and pin holes. First barrier layer 130 and second barrier layer 131 may be applied on the opposite side to provide the desired barrier properties in the finished material, such as grease resistance, water barrier and heat resistance.

The examples that follow are intended to illustrate the invention and not to limit it. All percentages used herein are by weight unless otherwise indicated.

### EXAMPLE

### EXAMPLE 1: Preparation of Coatings

Coatings were prepared with the types and amounts of components described below.

**Coating A: (46.3% solids)**

| Component | Amount (kg) |
|---|---|
| Acrylic Emulsion | 867 |
| Talc (dry powder) | 124 |
| Synthetic Defoamer | 5.0 |
| Dispersing Aid | 1.3 |
| Synthetic Thickener | 3.3 |

**Coating B: (56% solids)**

| Component | Amount |
|---|---|
| Acrylic Emulsion | 779 |
| Talc (dry powder) | 160 |
| Synthetic Defoamer | 4.4 |
| Dispersing Aid | 1.9 |

**Coating C: (60% solids)**

| Component | Amount |
|---|---|
| Styrenebutadiene dispersion | 1000 |

### EXAMPLE 2: Preparation of Grease and Moisture Resistant Coated Paperboard

Paperboard, Strom-baseboard 231g/m², produced at Stromdal's board machine is supplied to an off-line coating machine. The paperboard is coated with Coating A described in Example 1 at coating weight of 8 g/m² (coating weights are expressed as dry weight). The coated paperboard is dried with hot air at a temperature of 260°C for about 0.4 seconds to provide a web temperature of 70-90°C. After Coating A has been applied, Coating B as described in Example 1 is applied at the next coating station using the same procedure as used for applying Coating A. Coating B is applied a rate of 7 g/m². The coated paperboard is dried with hot air at a temperature of 500°C for about 0.4 seconds, then followed by drying with hot air at temperature of 160°C for about 4 seconds. After this the web temperature reaches temperature of 100-108°C. The coated and dried paperboard substrate is cooled by contacting the substrate with a roller having a temperature of 30-40°C and cool air so that the web temperature reaches 30-40°C before reeling the paperboard web in a Pope reeler. The topside is coated with the printable pigment coating. The cooled substrate is calandered by passing the substrate through rollers having nip pressure 40kN/m and temperature of 160°C. Coating layer A provides the paperboard with a grease penetration of 0 after 15 minutes at an oven temperature of 200°C. Coating layer B provides a moisture barrier. Water resistance is below 10g/m² measured with Cobb water absorption test (time 30 minutes). The resulting coated paperboard has surface properties that make it effective for further processing, such as for example in heat sealable, non-blocking uses. The coating withstands oven temperature of 220°C without loosing its barrier properties. Further, any substances in the coating do not migrate to the food in contact with the coating. At the same time, the coating is heat sealable with pressure of 80-100psi (551-689 kPa) and temperature of 160-200°C and time 1-1.5 seconds. As used herein, "heat sealable" refers to material that seals under pressure and elevated temperature without adhesives and which results in fiber tear when two heat sealable surfaces are separated. The coating can also be glued with waterbased glues without perforating the surface or any need for corona treatment as needed with traditionally used extruded polyolefines like PE-coatings.

### EXAMPLE 3: Preparation of Paper Board with Moisture Barrier and Grease Resistance

Paperboard is supplied to a coating machine. The paperboard is coated with Coating C described in Example 1 at rate of 8 gsm. The coated paperboard is dried at a temperature of 200°C for about 0.4 seconds. Coating B as described in Example 1 is then applied at the next coating station using the same procedure as used for applying Coating C. Coating B is applied at a of 7 g/m². The coated paperboard is dried with hot air at a temperature of 500°C for about 0.4 seconds, then followed by drying with hot air at temperature of 160°C for about 4 seconds. After this the web temperature reaches temperature of 100-108°C. The coated and dried paperboard substrate is cooled by contacting the substrate with a roller having a temperature of 30-40°C and cool air so that the web temperature reaches 30-40°C before reeling the paperboard web in a Pope reeler. The topside is coated with the printable pigment coating. The cooled substrate is calandered by passing the substrate through rollers having nip pressure 40kN/m and temperature of 160°C. Coating layer C provides a moisture vapour resistance (MVTR) of below 35 g/m². Coating layer B provides the paperboard with a heat sealability and water resistance, which is below 10 g/m² measured with Cobb water absorption test (time 30 minutes). The combination of these two coating layers provides grease penetration of 0 after 15 minutes at an oven temperature of 200°C. The resulting coated paperboard has surface properties that make it effective for further processing, such as for example in heat sealable, non-blocking uses. The coating withstands oven temperature of 220°C without loosing its barrier properties. Further, any substances in the coating do not migrate to the food in contact with the coating. At the same time, the coating is heat sealable with pressure of 80-100psi (551-689 kPa) and temperature of 160-200°C and time 1-1.5 seconds. As used herein, "heat sealable" refers to material that seals under pressure and elevated temperature without adhesives and which results in fiber tear when two heat sealable surfaces are separated. The coating can also be glued with waterbased glues without perforating the surface or any need for corona treatment as needed with traditionally used extruded polyolefines like PE-coatings.

Two layers of coating color, 11 g/m² each, are applied on the opposite side of the paperboard. Pigments are mainly calcium carbonate, but also clay is used on the top coat layer. The pigment coatings are applied with the same coating stations, but blades are used instead of rods or grooved rods to meter the needed coating weight and have even coating surface.

### EXAMPLE 4: Baking Test

Baking test is done for a 10x10cm sample of coated paperboard. Butter pastry is placed on coated side and baked at 200°C for 15 minutes. After cooling (5 minutes) the grease penetration through the coating is checked from the uncoated side of the board. Scale is 0-5, where 0 means no grease penetration.

**Evaluation scale**

| Value | Penetration of the grease in uncoated side |
|---|---|
| 0: | No grease penetration |
| 1: | couple of grease spots |
| 2: | several spots |
| 3: | <50% of the area |
| 4: | >50% of the area |
| 5: | Whole area |

## Claims

1. A method for producing coated recyclable paper or paperboard, wherein the paper or paperboard is coated with at least a first and second coating layers consisting of an aqueous polymer dispersion, **characterized in that**:
- the aqueous polymer dispersion in each layer consists of from about 70 to about 90 weight % of a polymer emulsion based on the dry weight of the coating and from about 10 to about 30 weight % of a pigment based on the dry weight of the coating with any remainder consisting of additives selected from the group consisting of thickening agents, de-foaming or antifoaming agents, dispersing aids, crosslinking agents, slip additives, release agents and antiblocking agents, with no waxes present;
and **in that** the method of coating comprises the steps of:
a) drying each coating layer to an elevated temperature by applying heated air having a temperature above about 100°C; and
b) cooling the coated paper or paperboard to a temperature below about 40°C;
wherein the drying and cooling steps (a) and (b) result in the coated paper or paperboard product having a water resistance of less than 10 g/m² and a moisture vapor transfer rate of less than 120 g/m², and wherein the coated paper or paperboard product is heat sealable.

2. The method of claim 1, wherein the coating operation occurs off-line from the manufacture of the paper or paperboard in the same facility as the paper or paperboard manufacturing system or in a different facility.

3. The method of claim 1 or 2, wherein the aqueous polymer dispersion is applied on the paper or paperboard having a temperature of 40°C or less.

4. The method of claim 3, wherein cooling step (b) is accomplished by air cooling or by containing the coated paper or paperboard within a cooling cylinder having a temperature of 40°C or less.

5. The method of claim 1 or 4, wherein the aqueous polymer dispersion has a viscosity of about 400 to about 1000 mPas and a solids content of about 40 to about 60 weight percent, based on the weight of the coating.

6. The method of claim 1 or 5, wherein the aqueous polymer emulsion is selected from the group consisting of acrylic polymers, acrylic copolymers, copolymers of styrene and butadiene, vinyl acetate polymers, polyvinyl alcohol, polyethylene vinyl acetate emulsions, and mixtures thereof.

7. The method of claim 6, wherein the acrylic polymer emulsion is selected from the group consisting of ethylacrylate, methylmethacrylate, butylacrylate, 2-ethylhexylacrylate, methylacrylate, ethylmethacrylate emulsions, and mixtures thereof.

8. The method of claim 6, wherein the aqueous polymer emulsion is an acrylic emulsion or a styrenebutadiene emulsion.

9. The method of claim 6 or 8, wherein the pigment is selected from the group consisting of aqueous dispersions of coating grade clays, titanium dioxide, calcium carbonate, barium sulfate, talc, zinc sulfate, aluminum sulfate, calcium oxide reaction products, lithopone, zinc sulfide, and mixtures thereof.

10. The method of claim 9, wherein the pigment is talc.

11. The method of any of the preceding claims, wherein each coating layer is formed using a rod or a bar with between about 5 g/m² to about 10 g/m² of aqueous coating.

12. The method of claim 11, wherein each coating layer is formed using a different aqueous polymer emulsion.

13. The method of claim 11 or 12, wherein at least one coating layer is applied to each side of the paper or paperboard.

14. The method of claim 12 or 13, wherein the first and second coating layer include a pigment selected from the group consisting of grade clays, titanium dioxide, calcium carbonate, barium sulfate, talc, zinc sulfate, aluminum sulfate, calcium oxide reaction products, lithopone, zinc sulfide, and mixtures thereof.

15. The method of claim 14, wherein the pigment is talc.

16. A coated paper or paperboard product having a baseboard layer with a coating thereon consisting of at least a first and second coating layers and being formed from an aqueous polymer dispersion, **characterized in that**:
- the aqueous polymer dispersion consisting for each coating layer from about 70 to about 90 weight % of a polymer emulsion based on the dry weight of the coating and from about 10 to about 30 weight % of a pigment based on the dry weight of the coating with any remainder consisting of additives selected from the group consisting of thickening agents, de-foaming or antifoaming agents, dispersing aids, crosslinking agents, slip additives, release agents and antiblocking agents with no waxes present;
- the coated paper or paperboard product possesses a water resistance of less than 10 g/m² and a moisture vapor transfer rate of less than 120 g/m² when the first and second coating layers are dried at an elevated temperature above about 100°C and the coating cooled to a temperature below about 40°C, whereby a coated paper or paperboard product is formed which is heat sealable.

17. The coated product of claim 16, wherein the first and second coating layers are formed from acrylic polymer emulsions which are selected from the group consisting of ethylacrylate, methylmethacrylate, butylacrylate, 2-ethylhexyl acrylate, methylacrylate, ethylmethacrylate emulsions, and mixtures thereof.

18. The coated product of claim 17, wherein the first and/or second coating layer(s) include(s) a pigment selected from the group consisting of grade clays, titanium dioxide, calcium carbonate, barium sulfate, talc, zinc sulfate, aluminum sulfate, calcium oxide reaction products, lithopone, zinc sulfide, and mixtures thereof.

19. The coated product of claim 18, wherein the pigment is talc.

20. The coated product of claim 16, wherein the first coating layer is formed from a styrenebutadiene emulsion, and the second coating layer contacts the first coating layer and is formed from an acrylic polymer emulsion.

21. The coated product of claim 20, wherein the acrylic polymer emulsion is selected from the group consisting of ethylacrylate, methylmethacrylate, butylacrylate, 2-ethylhexylacrylate, methylacrylate, ethylmethacrylate emulsions, and mixtures thereof.

## Patentansprüche

1. Verfahren zur Herstellung von beschichtetem, recycelbarem Papier oder Karton, bei dem das Papier oder der Karton mit wenigstens einer ersten und einer zweiten Beschichtungslage versehen wird, bestehend aus einer wäßrigen Polymerdispersion, **dadurch gekennzeichnet, daß** die wäßrige Polymerdispersion in jeder Lage aus einer etwa 70 bis etwa 90 Gew.-%igen Polymeremulsion besteht auf der Grundlage des Trockengewichts der Beschichtung und aus etwa 10 bis etwa 30 Gew.-% eines Pigmentes auf der Grundlage des Trockengewichtes der Beschichtung, und zwar mit einem beliebigen Rest, bestehend aus Additiven, ausgewählt aus der Gruppe, die sich zusammensetzt aus Dickungsmitteln, Entschäumungs- oder Antischaummitteln, Dispersionshilfen, Vernetzungsmitteln, Gleitzusätzen, Lösungsmitteln und Antisperrmitteln, bei nicht vorhandenen Wachsen; und ferner **gekennzeichnet dadurch, daß** das Verfahren der Beschichtung die folgenden Schritte aufweist:
a) Trocknen jeder Beschichtungslage bei einer erhöhten Temperatur durch Verwendung von erhitzter Luft, die eine Temperatur von etwa 100 °C aufweist; und
b) Kühlen des beschichteten Papiers oder Kartons auf eine Temperatur unter etwa 40 °C;
wobei der Trocknungsschritt und der Kühlungsschritt (a) und (b) das beschichtete Papierprodukt oder Kartonprodukt ergibt, das einen Wasserwiderstand von weniger als 10 g / m² und eine Dampffeuchtigkeit-Übertragungsmenge von weniger als 120 g / m² aufweist, und wobei das beschichtete Papier- oder Kartonprodukt hitzebeständig ist.

2. Verfahren nach Anspruch 1, **dadurch gekennzeichnet, daß** der Beschichtungsvorgang außerhalb der Herstellung des Papiers oder Kartons in derselben Einrichtung wie das Papier- oder Kartonherstellungssystem oder in einer anderen Einrichtung stattfindet.

3. Verfahren nach Anspruch 1 oder 2, **dadurch gekennzeichnet, daß** die wäßrige Polymerdispersion auf das Papier oder den Karton aufgetragen wird, und zwar bei einer Temperatur von 40 °C derselben oder geringer.

4. Verfahren nach Anspruch 3, **dadurch gekennzeichnet, daß** der Kühlungsschritt b) durch Luftkühlung oder dadurch bewirkt wird, daß das beschichtete Papier oder der beschichtete Karton in einem Kühlzylinder enthalten ist, der eine Temperatur von 40 °C oder weniger aufweist.

5. Verfahren nach Anspruch 1 oder 4, **dadurch gekennzeichnet, daß** die wäßrige Polymerdispersion eine Viskosität von etwa 400 bis etwa 1000 mPas und einen Feststoffgehalt von etwa 40 bis etwa 60 Gew.-%, auf der Grundlage des Gewichtes der Beschichtung, aufweist.

6. Verfahren nach Anspruch 1 oder 5, **dadurch gekennzeichnet, daß** die wäßrige Polymeremulsion ausgewählt wird aus der Gruppe, die besteht aus Acrylpolymeren, Acrylcopolymeren, Polymeren des Styrens und Butadien, Vinylazetatpolymeren, Polyvinylalkohol, Polyethylenvinylazetat-Emulsionen und deren Mischungen.

7. Verfahren nach Anspruch 6, **dadurch gekennzeichnet, daß** die Acrylpolymeremulsion aus der Gruppe ausgewählt wird, die besteht aus Ethylacrylat, Methylmethacrylat, Butylacrylat, 2-Ethylhexylacrylat, Methylacrylat, Ethylmethacrylat-Emulsionen und deren Gemische.

8. Verfahren nach Anspruch 6, **dadurch gekennzeichnet, daß** die wäßrige Polymeremulsion eine Acrylemulsion oder eine Styrenbuadien-Emulsion ist.

9. Verfahren nach Anspruch 6 oder 8, **dadurch gekennzeichnet, daß** das Pigment aus der Gruppe ausgewählt wird, die sich zusammensetzt aus wäßrigen Dispersionen von Beschichtungstonsorten, Titandioxid, Kalziumkarbonat, Bariumsulfat, Talk, Zinksulfat, Aluminiumsulfat, Kalziumoxid-Reaktionsprodukten, Lothopone, Zinksulfid und deren Gemische.

10. Verfahren nach Anspruch 9, **dadurch gekennzeichnet, daß** das Pigment Talk ist.

11. Verfahren nach einem der vorhergehenden Ansprüche, **dadurch gekennzeichnet, daß** jede Beschichtungslage durch Benutzung eines Stabes oder einer Stange zwischen etwa 5 g / m² bis etwa 10 g / m² des wäßrigen Bezugs geformt wird.

12. Verfahren nach Anspruch 11, **dadurch gekennzeichnet, daß** jede Beschichtungslage unter Verwendung einer anderen wäßrigen Polymeremulsion geformt wird.

13. Verfahren nach Anspruch 11 oder 12, **dadurch gekennzeichnet, daß** wenigstens eine Beschichtungslage für jede Seite des Papiers oder Kartons benutzt wird.

14. Verfahren nach Anspruch 12 oder 13, **dadurch gekennzeichnet, daß** die ersten und zweiten Beschichtungslagen ein Pigment enthalten, das aus der Gruppe ausgewählt ist, die besteht aus Tonmaterialien, Titandioxid, Kalziumkarbonat, Bariumsulfat, Talk, Zinksulfat, Aluminiumsulfat, KalziumoxidReaktionsprodukten, Lithopone, Zinksulfit und deren Gemische.

15. Verfahren nach Anspruch 14, **dadurch gekennzeichnet, daß** das Pigment Talk ist.

16. Beschichtetes Papier oder Kartonprodukt, das eine Bodenlage aufweist, auf der sich eine Beschichtung befindet, bestehend aus wenigstens einer ersten und einer zweiten Beschichtungslage und die gebildet ist aus einer wäßrigen Polymerdispersion, **dadurch gekennzeichnet, daß** die wäßrige Polymerdispersion für jede Beschichtungslage aus etwa 70 bis etwa 90 Gew.-% einer Polymeremulsion besteht, die auf dem Trockengewicht der Beschichtung beruht, und zwar von etwa 10 bis etwa 30 Gew.-% eines Pigments auf der Grundlage des Trockengewichtes der Beschichtung mit einem beliebigen Rest, bestehend aus Additiven, ausgewählt aus der Gruppe, die sich zusammensetzt aus Dickungsmittel, Entschäumungs- oder Antischaummittel, Dispersionshilfen, Vernetzungsmitteln, Gleitzusätzen, Lösungsmitteln und Antisperrmitteln, wobei keine Wachse vorhanden sind; ferner **dadurch gekennzeichnet, daß** das beschichtete Papier oder Pappeprodukt eine Wasserresistenz von weniger als 10 g / m² sowie eine DampffeuchtigkeitsÜbertragungsmenge von weniger als 120 g / m² aufweist, wenn die ersten und zweiten Beschichtungslagen bei einer erhöhten Temperatur von über etwa 100 °C getrocknet werden und die Beschichtung auf eine Temperatur unter etwa 40 °C gekühlt wird, wodurch ein beschichtetes Papier oder Kartonprodukt geschaffen wird, das wärmebeständig ist.

17. Beschichtetes Produkt nach Anspruch 16, **dadurch gekennzeichnet, daß** die ersten und zweiten Beschichtungslagen aus Acrylpolymeremulsionen gebildet sind, die aus der Gruppe ausgewählt sind, welche besteht aus Ethylacrylat, Methylmethacrylat, Butylacrylat, 2-Ethylhexylacrylat, Methylacrylat, Ethylmetacrylat-Emulsionen und deren Gemische.

18. Beschichtetes Produkt nach Anspruch 17, **dadurch gekennzeichnet, daß** die ersten und / oder zweiten Beschichtungslagen ein Pigment aufweisen, das aus der Gruppe ausgewählt ist, die aus Tonmaterialien, Titandioxid, Kalziumkarbonat, Bariumsulfat, Talk, Zinksulfat, Aluminiumsulfat, Kalziumoxid-Reaktionsprodukten, Lithopon, Zinksulfid und deren Gemischen besteht.

19. Beschichtetes Produkt nach Anspruch 13, **dadurch gekennzeichnet, daß** das Pigment Talk ist.

20. Beschichtetes Produkt nach Anspruch 16, **dadurch gekennzeichnet, daß** die erste Beschichtungslage aus einer Styrenbutadien-Emulsion gebildet ist und die zweite Beschichtungslage die erste Beschichtungslage berührt und aus einer Acrylpolymer-Emulsion gebildet ist.

21. Beschichtetes Produkt nach Anspruch 20, **dadurch gekennzeichnet, daß** die Acrylpolymer-Emulsion aus der Gruppe ausgewählt ist, die aus Ethylacrylat, Methylmethacrylat, Butylacrylat, 2-Ethylhexylacrylat, Methylacrylat, Ethylmetacrylat-Emulsionen und deren Gemischen besteht.

## Revendications

1. Procédé de production de papier ou de carton couché recyclable, dans lequel le papier ou le carton est revêtu au moins d'une première et d'une seconde couche de revêtement constituée par une dispersion polymère aqueuse, **caractérisé en ce que** :
- la dispersion polymère aqueuse dans chaque couche est constituée d'environ 70 à environ 90 % en poids, sur la base du poids sec du revêtement, d'une émulsion polymère et d'environ 10 à environ 30 % en poids, sur la base du poids sec du revêtement, d'un pigment, avec un éventuel reste constitué d'additifs choisis dans le groupe constitué par les agents épaississants, les agents suppresseurs de mousse ou antimousse, les aides à la dispersion, les agents de réticulation, les additifs de coulance, les agents de démoulage et les agents antibloquants, sans cires présentes ;
et **en ce que** le procédé de couchage comprend les étapes de :
a) séchage de chaque couche de revêtement à une température élevée par application d'un air chauffé ayant une température supérieure à environ 100°C ; et
b) refroidissement du papier ou du carton couché jusqu'à une température inférieure à environ 40°C ;
dans lequel les étapes de séchage et de refroidissement (a) et (b) donnent un produit de papier ou de carton couché ayant une résistance à l'eau inférieure à 10 g/m² et une vitesse de transfert de vapeur humide inférieure à 120 g/m², ledit produit de papier ou de carton couché étant thermoscellable.

2. Procédé selon la revendication 1, dans lequel l'opération de couchage est mise en oeuvre hors de la ligne de fabrication du papier ou du carton, dans la même unité de production que le système de fabrication du papier ou du carton ou dans une unité de production différente.

3. Procédé selon la revendication 1 ou 2, dans lequel la dispersion polymère aqueuse est appliquée sur le papier ou le carton ayant une température de 40°C ou moins.

4. Procédé selon la revendication 3, dans lequel l'étape de refroidissement (b) est réalisée par refroidissement par air ou par confinement du papier ou du carton couché dans un cylindre de refroidissement ayant une température de 40°C ou moins.

5. Procédé selon la revendication 1 ou 4, dans lequel la dispersion polymère aqueuse a une viscosité d'environ 400 à environ 1000 mPa.s et une teneur en fractions solides d'environ 40 à environ 60 % en poids, sur la base du poids du revêtement.

6. Procédé selon la revendication 1 ou 5, dans lequel l'émulsion polymère aqueuse est choisie dans le groupe constitué par les émulsions de polymères acryliques, de copolymères acryliques, de copolymères de styrène et de butadiène, de polymères d'acétate de vinyle, d'alcool polyvinylique, de polyéthylène-acétate de vinyle, et leurs mélanges.

7. Procédé selon la revendication 6, dans lequel l'émulsion de polymère acrylique est choisie dans le groupe constitué par les émulsions d'acrylate d'éthyle, de méthacrylate de méthyle, d'acrylate de butyle, d'acrylate de 2-éthylhexyle, d'acrylate de méthyle, de méthacrylate d'éthyle, et leurs mélanges.

8. Procédé selon la revendication 6, dans lequel l'émulsion polymère aqueuse est une émulsion acrylique ou une émulsion de styrène-butadiène.

9. Procédé selon la revendication 6 ou 8, dans lequel le pigment est choisi dans le groupe constitué par les dispersions aqueuses d'argiles de qualité couchage, le dioxyde de titane, le carbonate de calcium, le sulfate de baryum, le talc, le sulfate de zinc, le sulfate d'aluminium, les produits réactionnels de l'oxyde de calcium, le lithopone, le sulfure de zinc, et leurs mélanges.

10. Procédé selon la revendication 9, dans lequel le pigment est du talc.

11. Procédé selon l'une quelconque des revendications précédentes, dans lequel chaque couche de revêtement est formée à l'aide d'une tige ou d'une barre avec d'environ 5 g/m² à environ 10 g/m² de revêtement aqueux.

12. Procédé selon la revendication 11, dans lequel chaque couche de revêtement est formée à l'aide d'une émulsion polymère différente.

13. Procédé selon la revendication 11 ou 12, dans lequel au moins une couche de revêtement est appliquée sur chaque face du papier ou du carton.

14. Procédé selon la revendication 12 ou 13, dans lequel les première et seconde couches de revêtement contiennent un pigment choisi dans le groupe constitué par les argiles de qualité couchage, le dioxyde de titane, le carbonate de calcium, le sulfate de baryum, le talc, le sulfate de zinc, le sulfate d'aluminium, les produits réactionnels de l'oxyde de calcium, le lithopone, le sulfure de zinc, et leurs mélanges.

15. Procédé selon la revendication 14, dans lequel le pigment est du talc.

16. Produit de papier ou de carton couché comportant une couche de base portant un revêtement constitué au moins d'une première et d'une seconde couche de revêtement et étant formé à partir d'une dispersion polymère aqueuse, **caractérisé en ce que** :
- pour chaque couche de revêtement, la dispersion polymère aqueuse est constituée d'environ 70 à environ 90 % en poids, sur la base du poids sec du revêtement, d'une émulsion polymère et d'environ 10 à environ 30 % en poids, sur la base du poids sec du revêtement, d'un pigment, avec un éventuel reste constitué d'additifs choisis dans le groupe constitué par les agents épaississants, les agents suppresseurs de mousse ou antimousse, les aides à la dispersion, les agents de réticulation, les additifs de coulance, les agents de démoulage et les agents antibloquants, sans cires présentes ;
- le produit de papier ou de carton couché possède une résistance à l'eau inférieure à 10 g/m² et une vitesse de transfert de vapeur humide inférieure à 120 g/m², quand les première et seconde couches de revêtement sont séchées à une température élevée supérieure à environ 100°C et que le revêtement est refroidi jusqu'à une température inférieure à environ 40°C, moyennnant quoi est formé un produit de papier ou de carton couché qui est thermoscellable.

17. Produit couché selon la revendication 16, dans lequel les première et seconde couches de revêtement sont formées à partir d'émulsions d'un polymère acrylique qui sont choisies dans le groupe constitué par les émulsions d'acrylate d'éthyle, de méthacrylate de méthyle, d'acrylate de butyle, d'acrylate de 2-éthylhexyle, d'acrylate de méthyle, de méthacrylate d'éthyle, et leurs mélanges.

18. Produit couché selon la revendication 17, dans lequel la première et/ou la seconde couche(s) contien(nen)t un pigment choisi dans le groupe constitué par les argiles de qualité couchage, le dioxyde de titane, le carbonate de calcium, le sulfate de baryum, le talc, le sulfate de zinc, le sulfate d'aluminium, les produits réactionnels de l'oxyde de calcium, le lithopone, le sulfure de zinc, et leurs mélanges.

19. Produit couché selon la revendication 18, dans lequel le pigment est du talc.

20. Produit couché selon la revendication 16, dans lequel la première couche de revêtement est formée à partir d'une émulsion de styrène-butadiène, et la seconde couche de revêtement est en contact avec la première couche de revêtement et est formée à partir d'une émulsion d'un polymère acrylique.

21. Produit couché selon la revendication 20, dans lequel l'émulsion de polymère acrylique est choisie dans le groupe comprenant les émulsions d'acrylate d'éthyle, de méthacrylate de méthyle, d'acrylate de butyle, d'acrylate de 2-éthylhexyle, d'acrylate de méthyle, de méthacrylate d'éthyle, et leurs mélanges.
